

Oct. 10, 1950

R. H. JENKS ET AL

2,525,603

METHOD OF MAKING LEAD COATED COPPER

Filed Nov. 21, 1945



Richard H. Jenks  
Wilson Lynes  
by  
C. W. Booth, Townsend  
Miller & Weidner

Attn:

## UNITED STATES PATENT OFFICE

2,525,603

## METHOD OF MAKING LEAD COATED COPPER

Richard H. Jenks, Sauquoit, and Wilson Lynes, Westerville, N. Y., assignors to Revere Copper and Brass Incorporated, Rome, N. Y., a corporation of Maryland

Application November 21, 1945, Serial No. 630,100

1 Claim. (Cl. 117—114)

1

Our invention relates to articles having copper surfaces, such as sheet copper, coated with a thin layer of lead for improving the resistance of the copper to atmospheric and other forms of corrosion, and to methods of making such articles.

Heretofore, in coating copper surfaces with lead, it has been common practice to alloy the lead with a small amount of tin for insuring proper adherence of the coating to such surfaces. Applicants have found that in employing tin for this purpose pitting of the copper frequently occurs by corrosive action where pinholes exist in the lead coating as formed, or where the coating is locally accidentally removed by mechanical means such as scratches. Although the reason for such pitting heretofore has not been exactly understood, it is believed by applicants that it occurs because when the coating is applied some of the tin alloys with the surface portion of the copper to form on the latter a film of substantially binary copper-tin alloy, with the result that when pinholes in the lead coating exist, or the coating is removed mechanically at localized points, there are exposed both bare copper and this film, and, the bare copper being anodic to the film, the bare copper is pitted when the article is exposed to a corrosive medium.

Applicants have found that in place of tin the lead may be alloyed with cadmium for insuring satisfactory adherence of the lead to the copper, and that if the cadmium is properly proportioned to the lead such a film either is not formed or if formed is anodic to the bare copper, so that pitting of the bare copper does not occur as a result of pinholes or the like in the coating.

Applicants have found, however, that if it is attempted to apply according to prior methods a coating of lead containing cadmium, the cadmium in the lead bath rapidly oxidizes and is lost, forming a layer of cadmium oxide dross on the surface of the bath. This dross adheres superficially to the coating and mars its appearance. It furthermore tends to mix with the material of the coating layer to form cadmium oxide segregates therein which act seriously to reduce the corrosion resisting properties of the coating itself.

According to the present invention, the drossing of the lead-cadmium bath is effectively prevented by causing the bath to contain aluminum. As little as 0.001% aluminum will prevent drossing of the cadmium and the presence of cadmium oxides in the coating, the surface of the bath with this amount of aluminum remaining bright and clean. The amount of aluminum however should

2

not exceed its limit of solubility in either the molten or solidified bath material, which limit is about 0.1%, as otherwise metallic aluminum segregates may be introduced into the coating causing deterioration thereof by galvanic action. Preferably to insure satisfactory results about 0.005 to 0.05% aluminum is employed.

The aluminum may be compounded with the lead by melting the lead and raising its temperature to at least about 1300° F., whereupon the aluminum may be added and the bath stirred. The cadmium may be added to the lead following the addition thereto of the aluminum. Preferably, however, the lead-aluminum alloy is cast into billets, and the cadmium is added when the billets are melted in the lead pot to form the coating bath which preferably is at a temperature between 825 and 875° F., this temperature however not being critical but being merely high enough to cause the bath to have sufficient fluidity properly to spread over the copper surface of the article when applied thereto to form thereon a thin coating of the lead alloy of from about 0.001 to 0.01 of an inch in thickness.

Applicants also have found, that unless suitable precautions are taken in respect to the amount of cadmium incorporated in the lead, the coating itself will be subject to serious deterioration when subjected to the action of a corrosive medium. It has been found that the amount of cadmium incorporated should be such as to result in the coating having a substantially single alloy phase structure. A plural alloy phase structure, because it in effect consists of an intimate mixture of different metal alloys, causes the occurrence of galvanic action on the coating itself when subjected to a corrosive medium, resulting in corrosion of the coating. This single phase structure, it has been found, will exist when the coating contains up to about 3.3% cadmium whether or not the aluminum is present, provided if the aluminum is present it is not substantially in excess of its limit of solubility in the lead.

With amounts of cadmium not in excess of about 3.3% the existence of a single phase structure apparently, for all practical purposes, is independent of the rate of cooling of the coating after it is applied in liquid state to the copper, the phase structure of the thin coating not being affected by rapid cooling of the coating as it passes from a temperature between the liquidus and solidus to a temperature below the solidus, which is not the case with lead-cadmium alloys of considerable mass or thickness. With amounts of cadmium in excess of about 3.3% the solidified coat-

ing will have a plural phase structure, characteristically a so-called "alpha-beta" structure, no matter at what rate it is cooled from any higher temperature to any lower temperature within the range of from any temperature at which it is liquid down to room temperatures. With amounts of cadmium less than 3.3% the coating has substantially wholly a so-called "alpha" structure.

To secure proper results from the cadmium at least about 0.5% thereof should be incorporated in the lead, and for the reasons above stated no more than about 3.3% thereof should be present. To insure satisfactory results preferably about 0.5 to 1% cadmium is employed.

Preferrably the coating is applied by dipping the article into the bath, with the latter at about 850° F. so that it will be highly fluid, whereupon the article is removed vertically from the bath to permit the excess of the coating to drain therefrom and the coating to spread uniformly over the copper surface. After the article is removed from the bath the coating may be permitted to cool, say by exposing it to air at room temperature or by subjecting it to a draft of air or to air jets.

The copper surface to be coated is, if necessary, first cleaned, and preferably fluxed before immersing the article in the bath. The cleaning of the copper may be effected by any suitable means, for example, by so-called "scratch brushing." The flux may be applied in liquid form at room temperature or slightly above, a suitable flux consisting of the addition to water of ammonium chloride and hydrochloric acid in the proportion of two pounds ammonium chloride and one gallon technical hydrochloric acid to one gallon water, the hydrochloric acid being added after the ammonium chloride is dissolved. Other acid fluxes may be employed, for instance, either aluminum chloride or cadmium chloride may be substituted for the ammonium chloride in this example. Also a thin coating of oil or the like is preferably applied to the fluxed copper surface for insuring against oxidation of such surface prior to the article being immersed in the lead bath. Palm oil, rapeseed oil, tallow, petroleum jelly and various petroleum oils may be employed for this purpose. It will be understood that cleaning the copper and fluxing and oiling it act to insure a continuous lead coating and good adherence of the same, but may not in all cases be necessary depending upon the condition of the copper surface to be treated and, if it is necessary to clean it, the time that must elapse between the cleaning operation and the emersion of the article in the bath.

Suitable apparatus for applying the coating to sheet copper is illustrated by the accompanying drawings in which:

Fig. 1 is a more or less diagrammatic vertical longitudinal section of the apparatus;

Fig. 2 is a plan of the flux and oil applying instrumentalities;

Fig. 3 is a plan of the instrumentality for cooling the coated sheet; and

Fig. 4 is a plan of the lead tank with parts omitted.

As shown in the drawings, the copper sheet S successively passes through a body of liquid flux in a tank 1, through a body of palm oil in a tank 3, through a bath of molten lead in a pot 5, and through an air box 7.

As illustrated, the flux and palm oil are maintained in the tanks 1 and 3 at levels 9, the sheet being guided through the body of flux and palm oil by spaced curved guide bars 11 below the sheet

and idle guide rolls 13 above the sheet. Steam coils 15 may be submerged in the flux and palm oil beneath the guide bars 11 for slightly heating these substances if necessary or desired. At the 5 exit ends of the flux and palm oil tanks 1 and 3 the sheet passes between pairs of driven wiper rolls 17 for removing excess flux and oil therefrom and advancing the sheet, which excess drains back into the tanks. At the entrance end of the 10 palm oil tank 3 the sheet passes between a pair of driven offset rolls 18 which deflect the sheet into the palm oil tank 3.

As shown, the lead pot 5 at a pair of opposite sides thereof is supported by beams 19 resting on 15 the opposite walls 21 of a furnace chamber into which the lead pot extends. Below the lead pot are provided gas burners 23 for heating the contents of the pot. As shown, the bath is maintained in the lead pot at a level 25, the sheet being 20 deflected into the bath by driven offset rolls 27. The sheet is guided through the bath in the lead pot by the spaced curved guide bars 29 positioned above the sheet and the spaced curved guide bars 31 positioned below the sheet. At the exit 25 side of the bath is provided an idle roll 33 adapted to engage the upper side of the sheet for assisting in guiding it in a vertical direction in which it is drawn by driven guide rolls 35 at the top of the air box 7, between which rolls 35 it passes after 30 traveling through said box, these rolls 35, like the rolls 17, 18 and 27, acting to advance the sheet.

In the air box 7 the sheet is cooled for hardening the coating sufficiently to prevent the rolls 35 from injuring it. To this end the sheet in 35 the air box passes between vertical banks of spaced horizontally disposed compressed air conducting pipes 37 each provided with a row of spaced jet nozzles 39 for directing air toward 40 each of opposite sides of the sheet, thus subjecting the latter to an air draft for cooling the coating. Each of the horizontal pipes 37 is connected to and supplied with compressed air from a vertically arranged header 41. These headers are 45 severally connected through a regulating valve 43 to a common pipe 45 supplied with compressed air from a suitable source. By use of the valves 43 the force of the air jets on opposite sides of the sheet may be so regulated that the sheet will 50 not be forced laterally in either direction. Preferably however, to insure against the sheet striking the jet nozzles under untoward conditions, spaced curved vertically extending guard bars 47 are arranged in the air box at opposite sides 55 of the sheet between it and the nozzles, these bars being in offset relation to the nozzles so as not to interfere with the air jets discharging therefrom.

It will be understood that within the scope of 60 the appended claim wide deviations may be made from the herein described embodiments of the invention without departing from the spirit of the invention.

We claim:

The method of protecting the copper surface of an article against corrosion comprising coating it with an adhering alloy of single phase structure substantially free from tin and containing a material which forms with copper a copper alloy anodic to copper, that material being cadmium, by forming a bath of molten alloy substantially free from tin and consisting essentially of lead having dissolved therein not less than about 0.5% cadmium to insure such adherence, or more than about 3.3% cadmium to insure against the

coating having other than a single phase structure, and also having dissolved therein not less than about 0.001% aluminum to prevent drossing of the cadmium and inclusion of cadmium oxide segregates in the coating, or more than about 0.1% aluminum also to insure against the coating having other than a single phase structure, immersing the article in said bath to cause the bath alloy to adhere thereto, and withdrawing from the bath the article coated with such alloy.

RICHARD H. JENKS.  
WILSON LYNES.

## REFERENCES CITED

The following references are of record in the file of this patent:

## UNITED STATES PATENTS

|    | Number    | Name     | Date          |
|----|-----------|----------|---------------|
| 5  | 243,766   | Feeley   | July 5, 1881  |
|    | 1,126,484 | Kirby    | Jan. 26, 1915 |
|    | 1,760,603 | Milbring | May 27, 1930  |
| 10 | 2,052,363 | Snyder   | Aug. 25, 1936 |
|    | 2,196,855 | Dietloff | Apr. 9, 1940  |

## FOREIGN PATENTS

| Number  | Country       | Date          |
|---------|---------------|---------------|
| 528,558 | Great Britain | Oct. 31, 1940 |